

# UNITED STATES PATENT OFFICE.

JOHN A. REID, OF GULFPORT, MISSISSIPPI.

## SHOE-POLISH.

1,194,425.

Specification of Letters Patent. Patented Aug. 15, 1916.

No Drawing.

Application filed June 18, 1915. Serial No. 34,871.

*To all whom it may concern:*

Be it known that I, JOHN A. REID, a citizen of the United States, residing at Gulfport, in the county of Harrison and State of Mississippi, have invented new and useful Improvements in Shoe-Polish, of which the following is a specification.

This invention relates to improvements in shoe polish and more particularly to a material for cleaning or recoloring shoes of light colored canvas, cloth, or leather.

It is the object of this invention to provide a material in powder form to be applied to soiled light colored shoes of fabric or leather for the purpose of cleaning or applying a coating of the material and thereby causing the shoes to assume their original color.

The advantages of this polish or material are that shoes of white, Palm Beach color, or gray color which quickly become soiled are readily cleaned or brought back to their original color by an application of this powder. The powder is dry and there is no loss to the user by evaporation as in liquid preparations of this character, and as the powder is applied dry there is no necessity of addition of water or other liquid which may not always be at hand, and there is no danger of discoloring other articles by accident when cleaning or recoloring the shoes as the powder may be brushed off at once.

It is preferable to place the powder in fabric bags of such texture that the powder may readily pass therethrough so that it may be readily applied by rubbing the shoes briskly with the bag. The fabric of the bag removes dirt attached to the shoe and the

powder passing through the fabric of the bag forms a coating over the surface of the 40 shoe.

The following ingredients combined in the following amounts will produce enough powder to fill a gross of bags for cleaning or recoloring white shoes. Spanish whiting, 7.5 45 pounds, oxid of zinc, 2.5 pounds, pumice stone, 1.5 pounds, granulated sugar, 1.5 pounds, flour, 3 pounds.

In preparing the powder for use upon Palm Beach shoes 1.6 pounds of yellow ocher 50 is added to the white material and for gray shoes 1.6 pounds of lamp black is added to the white material.

During the use of the bag the grains of the granulated sugar rub against each other 55 and the other ingredients which rubs off some of the sugar in powder form and imparts a sufficient amount of the sugar to the other ingredients to perform its function. Powdered sugar may be used in the first 60 place, if desired.

What I claim is:—

1. A shoe cleaning or recoloring powder comprising Spanish whiting 7.5 pounds, oxid of zinc 2.5 pounds, pumice stone 1.5 pounds, 65 sugar 1.5 pounds, flour 3 pounds.

2. A shoe cleaning or recoloring powder comprising Spanish whiting 7.5 pounds, oxid of zinc 2.5 pounds, pumice stone 1.5 pounds, sugar 1.5 pounds, flour 3 pounds, and color- 70 ing matter 1.6 pounds.

JNO. A. REID.

Witnesses:

EUGENE FLY,  
C. L. WALLER.